

1

2,965,459

## GASOLINE CONTAINING BORATED OXAZOLINES

Richard J. De Gray, Shaker Heights, and Sarah H. Belden, Cleveland, Ohio, assignors to The Standard Oil Company, Cleveland, Ohio, a corporation of Ohio

No Drawing. Filed Feb. 25, 1959, Ser. No. 795,349

Claims priority, application Great Britain Mar. 3, 1958

4 Claims. (Cl. 44—63)

This invention relates to novel compounds comprising borated oxazolines, the process for preparing these compounds, and gasoline containing the same. In particular, this invention relates to a class of novel boron compounds for use in gasoline which are prepared by reacting boric acid or boric oxide with a substituted oxazoline compound having the following general formula:



wherein  $R_x$  represents a saturated or unsaturated hydrocarbon, preferably an aliphatic hydrocarbon radical, containing 7 to 19 carbon atoms, and where  $R_y$  represents the radical  $-(CH_2)_nOH$  where  $n$  is a small whole number such as 1 to 3, and where  $R_z$  represents a radical selected from the group consisting of  $R_y$ , hydrogen, or a lower alkyl radical having 1 to 3 carbon atoms.

When  $R_z$  is  $R_y$ , the compounds will have the formula:



where  $X$  is hydrogen or



When  $R_z$  is hydrogen or an alkyl radical, the compounds have the formula:



It is well known in the prior art that the continued operation of the internal combustion engine results in the formation of combustion chamber deposits. This deposit problem is particularly aggravated when tetraethyl lead is contained in the fuel for the purpose of increasing the octane number of the fuel to a desired level for modern high-compression engines. The use of leaded fuels leaves combustion chamber deposits which are no longer essentially carbonaceous in chemical nature, but comprise appreciable quantities of lead compounds generally mixed in the carbonaceous material. The fact that such deposits are partially metallic in character is believed to give it a catalytic activity which modifies the action of the deposit in affecting engine operation. Despite the fact that one or more volatile organic halides

2

such as ethylene dichloride and/or ethylene dibromide are included in the fuel as scavenging agents, not all the lead is removed.

Combustion chamber deposits, and particularly deposits resulting from the burning of leaded fuels, produce a number of adverse effects in engine operation, notable among which is a tendency for these deposits to become heated to incandescence, developing one or more hot spots in the combustion chamber. These spots ignite the fuel either before or after the position in the cycle at which the fuel would normally be ignited by the spark of the sparkplug. This condition, referred to commonly as surface ignition, manifests itself in various ways characterized as different forms of knocking or engine roughness, and usually resulting in appreciable power loss.

It has already been proposed that the introduction of organo boron compounds into a gasoline serves to alleviate the adverse effects of combustion chamber deposits either by the removal of some of these deposits or by altering such deposits to increase the efficiency of combustion in the combustion chamber of the engine. However, many organo boron compounds are not sufficiently stable or adequately soluble and stable in gasoline to be suitable for commercial use. The boron compounds of this invention, in contradistinction to many other classes of organo boron compounds, are liquids that are highly resistant to crystallization in their pure form even when exposed to very humid atmospheric conditions. Consequently, they may be prepared well in advance of the time when it is required for them to be incorporated into gasoline and may be blended into gasoline without any special precautions to avoid contact with moisture. Furthermore, these boron compounds, when dissolved in gasoline, exhibit excellent stability toward hydrolysis, enabling them to be satisfactorily used in large scale manufacturing and marketing operations where the gasoline containing the boron compound must be placed in storage tanks at bulk stations, at filling stations, and in individual cars, all of which normally contain small amounts of water at the bottom thereof. It will be obvious that unless the boron compound is hydrolytically stable, the contact of the gasoline with such water bottoms will gradually result in the hydrolysis of the boron compound, resulting in the formation of boric acid or other compound forms which precipitate from the hydrocarbon phase to the water phase that is present and the additive is lost for any benefit in the combustion chamber. Solid precipitates forming from such unstable compounds may also clog fuel lines and filters or otherwise interfere with the operation of the engine.

In addition to overcoming in great part the adverse effects due to combustion chamber deposits, the motor fuels of the present invention are also found particularly helpful in preventing carburetor deposits. Harmful deposits commonly accumulate in the carburetors of motor vehicles operating in urban areas from contaminated intake air which the carburetor must breathe in in tremendous volumes for engine operation, manifesting themselves by causing rough idling of the engine and in many cases the occurrence of frequent stalling.

The major contributor to this responsible contamination in the air is believed to be the combustion products exhausted from the large population of other cars operating in the same immediate area. The condition is, of course, aggravated by any blowby fumes from the operation of the car's own engine or by any other under-hood fumes generated by the car's engine, in addition to any industrial fumes present in the air which the carburetor breathes. These sources of contamination are additive in nature and may cause the rapid build-up of deposits on the carburetor of the engine.

The motor fuels of the present invention are further characterized by their effectiveness in minimizing carburetor icing. The latter condition represents another troublesome problem attendant to automotive engines operated in cool, moist, atmospheric conditions. This icing problem is most likely to occur during engine warm-up when the engine is below normal operating temperature. Vaporization of the gasoline in the carburetor during this warm-up period produces temperature reduction of the throttle plate and carburetor walls, causing the moisture present in the incoming air on cool, humid days to condense and freeze. Such ice formation restricts the narrow openings in the carburetor, manifesting itself in a rough idling condition and frequent engine stalls.

Furthermore, the boron compounds of this invention, when present in small amounts in a motor fuel, are highly effective as anti-rust agents.

The above beneficial effects are gained when the boron compounds of this invention are incorporated in a gasoline in amounts between 0.0025 to 0.05% by weight, with amounts from 0.02 to 0.05% by weight being preferred.

The substituted oxazoline compound used in preparing the boron compounds of this invention may be prepared from amino hydroxy compounds through their fatty amides, or any other known procedure. In preparing these oxazolines from the fatty acid amides, a suitable amino hydroxy compound is reacted with a desirable fatty acid, or a mixture thereof, at an elevated temperature to yield the amide. The temperature is then increased so as to split out water and form the oxazoline.

Any of the compounds having the general formula offered above are suitable for the invention. The preferred compounds, however, are those in which  $R_x$  as defined heretofore contains 11 to 17 carbon atoms for maximum solubility in hydrocarbon fuel and where  $R_z$  is the equivalent of  $R_y$ . Mixtures of compounds may be used as  $R_x$ , and this frequently will be the case since the  $R_x$  radical is derived from naturally occurring fats and oils, and hence  $R_x$  will correspond to the fatty acid radicals in such fats and oils, such as tallow, cottonseed oil, soybean oil, tall oil, etc. The nature of  $R_x$  does not affect the results appreciably, it has been found, and therefore its selection will be dictated largely by economics. The commercial grade of the compounds, including small amounts of impurities or by-products, are suitable. A particularly desirable compound for purposes of the invention is 2-heptadecenyl 4,4-bis-(hydroxy methyl) oxazoline and has the formula:



These substituted oxazolines readily undergo reaction with boric acid under conditions in which the water of reaction may be removed from the reaction mixture as it is formed. This removal of water may be accomplished by simple boiling, but it is preferable to remove the water by means of azeotropic fractional distillation. Boric oxide may be used in place of boric acid in these reactions with only the requirement for making the appropriate weight adjustment in order to maintain the molar relationship with the substituted oxazoline.

The preparation of these compounds will be better understood in connection with the following example in which the substituted oxazoline is 2-heptadecenyl 4,4-bis-(hydroxy methyl) oxazoline but which is typical of the reaction with other substituted oxazolines of the general formula previously designated. The parts referred to in the examples are parts by weight unless otherwise noted.

## EXAMPLE 1

100 parts of 2-heptadecenyl 4,4-bis-(hydroxy methyl) oxazoline was dissolved in 200 parts of benzene. 16.8 parts of boric acid was then added (a 1:1 molar ratio) and the mixture refluxed at the azeotropic distillation temperature for the removal of water with the benzene overhead from the reaction mixture. The remainder of the benzene was distilled off. The reaction proceeds readily in accordance with the following equation:



The reaction product was a clear liquid upon cooling and was soluble in gasoline.

## EXAMPLE 2

50 parts of 2-heptadecenyl 4,4-bis-(hydroxy methyl) oxazoline was dissolved in 100 parts of benzene. 8.4 parts of dry boric acid was then added (a 1:1 molar ratio) and the mixture refluxed for several hours at the azeotropic distillation temperature for the removal of water overhead. The reaction proceeds in accordance with the following equation:



The remainder of the benzene was distilled off and the compound of this example, upon cooling to room temperature, was a clear liquid and soluble in gasoline. The recovery of the water of reaction showed that two and one-half mols of water were formed for each mol of 2-heptadecenyl 4,4-bis-(hydroxy methyl) oxazoline and boric acid reacting.

The compound of this example can also be prepared from the compound of Example 1 by further dehydration of the latter according to the equation:



## EXAMPLE 3

100 parts of 2-heptadecenyl 4-methyl, 4-hydroxy methyl oxazoline was dissolved in 200 parts of benzene. 8.8 parts of boric acid was then added (a 2:1 molar ratio) and the mixture was refluxed at the azeotropic distillation temperature for the removal of water with benzene overhead. The remainder of the benzene was

distilled off. The reaction proceeds according to the following equation:



The reaction product was a clear liquid at room temperature and was soluble in gasoline.

The motor fuel consists essentially of one or more hydrocarbon base stocks which may be any of those conventionally used in preparing a motor gasoline for a spark-ignited internal combustion engine, such as catalytic distillate, motor polymer, alkylate, catalytic reformat, isomerate, naphthas, etc., and one or more of the above-defined compounds. It is intended that the gasoline of the invention may also contain tetraethyl lead in amounts up to 6 ml., generally up to 3 ml., but at least  $\frac{1}{2}$  ml. per gallon and a scavenging agent. This definition permits the inclusion, in addition to the lead anti-detonant and a scavenger composition, of antioxidants, stabilizers, solvent oils, dyes, other additives such as boron compounds, phosphorus compounds, and the like.

A clearer understanding of the benefits derived from the fuel of this invention will be obvious from the results obtained from the following testing program.

#### Surface ignition suppression

To determine the effectiveness of the gasoline of this invention to suppress surface ignition, an ASTM-CFR single-cylinder engine having the compression ratio adjusted at 12:1 was employed. Preparatory to the test cycle, the engine was run open throttle at 900 r.p.m. for thirty minutes to stabilize the engine conditions for the test period. Following this, the engine was continued at open throttle continuously for three hours, during which time the total surface ignition count was observed electronically. All experimental conditions were the same for each test except the gasoline.

The base fuel in each test was the same and had the following composition and specifications:

#### Composition:

|                             |          |      |
|-----------------------------|----------|------|
| Ultraformate                | percent  | 59.8 |
| Catalytic distillate        | do       | 30.0 |
| Light naphtha               | do       | 10.0 |
| Solvent oil                 | do       | 0.2  |
| Tetraethyl lead (motor mix) | ml./gal. | 3.0  |
| API gravity                 |          | 49.7 |

#### Engler distillation:

|     |      |     |
|-----|------|-----|
| IBP | ° F. | 80  |
| 10% | ° F. | 155 |
| 30  | ° F. | 202 |
| 50  | ° F. | 263 |
| 70  | ° F. | 310 |
| 90  | ° F. | 377 |
| EP  | ° F. | 452 |

Reid vapor pressure 6.5

The number of surface ignitions in the additive fuel is expressed as percentage of the surface ignitions of the blank fuel with the results as follows:

| Additive              | Concen-<br>tration,<br>percent<br>by wt. | SI Rating of Fuel |               |
|-----------------------|------------------------------------------|-------------------|---------------|
|                       |                                          | Total SI          | Audible<br>SI |
| None                  | None                                     | 100               | 100           |
| Compound of Example 1 | 0.02                                     | 59                | 56            |
| Compound of Example 1 | 0.05                                     | 26                | 42            |

#### 10 Carburetor cleanliness

A test was devised to determine an effective rating for promoting carburetor cleanliness with the gasoline of the invention as compared with the same gasoline not containing an oxazoline compound. In this test a contamination system was developed to simulate the conditions which contribute to carburetor deposits in the urban operation of motor vehicles. The system comprises the operation of a slave engine and a test engine. The exhaust gases from one bank of the slave engine (four cylinders) is metered to the crankcase of the test engine at a rate of 1.5 cubic feet per minute. All gases from the crankcase of the test engine are passed to the air intake of the carburetor of the test engine including, therefore, the exhaust gases from the slave engine and the blowby fumes of the test engine. The 1.5 cubic feet per minute rate of exhaust gases from the slave engine under these conditions constitutes approximately 8% of the total air intake of the test engine at idle manifold vacuum and speed. The operating conditions for the two engines are as follows:

|                  | Test Engine                                                                                      | Slave Engine                            |
|------------------|--------------------------------------------------------------------------------------------------|-----------------------------------------|
| Engines          | '54 Olds, 10; 1 C.R.                                                                             | '55 Chrys, 11; 1 C.R.                   |
| Spk. Plugs       | Champion J-12                                                                                    | Champion N-8B.                          |
| Carburetion      | Standard four-barrel Rochester carburetor.                                                       | Standard four-barrel Carter carburetor. |
| Eng. Speed       | Set up initially for each test at 850 r.p.m. except for accelerations to 3,000 r.p.m., unloaded. | 700 r.p.m. $\pm$ 20.                    |
| 40. Jacket Temp. | 160° F. $\pm$ 5°                                                                                 | 165° F. $\pm$ 5°                        |

The test cycle was 2 hours in time, which included four acceleration periods conducted on the unloaded test engine spaced at  $\frac{1}{2}$  hour intervals, the first acceleration period being 30 minutes after the test cycle was commenced. During each acceleration period the throttle was moved quickly to a wide open position and then quickly closed again to an idle position five separate times to permit a surge of carburetted gasoline to come into contact with the carburetor parts. The carburetor at the start of each test was in spotless condition. All experimental conditions were the same for the two test cycles except for the gasoline.

The base fuel in each test was the same and had the following composition and specifications:

|              |                 |         |      |
|--------------|-----------------|---------|------|
| Composition: | Cat. distillate | percent | 75   |
|              | SR naphtha      | do      | 25   |
|              | API gravity     |         | 62.4 |

|                      |                     |      |      |
|----------------------|---------------------|------|------|
| Engler distillation: | IBP                 | ° F. | 98   |
|                      | 10%                 | ° F. | 130  |
|                      | 30                  | ° F. | 163  |
|                      | 50                  | ° F. | 204  |
|                      | 65                  | ° F. | 262  |
|                      | 70                  | ° F. | 365  |
|                      | 90                  | ° F. | 424  |
|                      | EP                  | ° F. | 8.75 |
|                      | Reid vapor pressure |      |      |

At the end of each test the carburetor was removed and disassembled and a numerical rating was assigned for amount of deposits and discoloration by a number of observers rating independently and uninformed of the gasoline they were rating. The rating assigned was based on a standardized scale ranging from 100 to 0,

wherein 100 would be a rating of a perfectly clean carburetor throttle plate and barrel, and 0 rating would represent a throttle plate and barrel loaded with deposits.

The results below represent the average rating by the observers:

| Additive              | Concen-<br>tration,<br>percent<br>by wt. | Rating |
|-----------------------|------------------------------------------|--------|
| None                  | None                                     | 60     |
| Compound of Example 1 | 0.0025                                   | 78     |
| Compound of Example 1 | 0.02                                     | 83     |

#### Carburetor anti-icing

A test procedure was devised simulating the stop-and-go type of engine operation normally experienced by the motorist during the engine warmup period. The test was conducted in a 1955 Plymouth V-8 engine equipped with a two-barrel carburetor. Carburetor air was supplied at a constant rate of 70 cubic feet per minute by a specially designed air conditioner controlled at 42° F. and 90% relative humidity, which are temperature and humidity conditions considered highly conducive to carburetor icing. All test conditions were the same except for the gasoline.

The test consisted of running the same number of cycles on each fuel where in each cycle the engine was operated at 2200 r.p.m. for 15 seconds and then decelerated normally to an idle at 450 r.p.m. for a maximum of 30 seconds. Performance of the engine was observed during each idle period, and a numerical rating based on the degree of rough idling and engine stalls was assigned so that each fuel received a merit rating on a scale ranging from 100 to 0. By this scheme an engine operating with a smooth idle over the idle periods of every test cycle would receive a rating of 100, and an engine which stalled in less than 12 seconds in the idle period of every test cycle would receive a rating of 0.

The base fuel used had the following composition and specifications.

#### Composition:

|                             |          |      |
|-----------------------------|----------|------|
| Lt. cat. distillate         | percent  | 48.5 |
| Ultraformate                | do       | 28.9 |
| Lt. naphtha                 | do       | 9.7  |
| Isopentane                  | do       | 4.9  |
| Butane                      | do       | 7.8  |
| Solvent oil                 | do       | 0.2  |
| Tetraethyl lead (motor mix) | ml./gal. | 3.0  |
| API gravity                 |          | 61.7 |

#### Engler distillation:

|                     |      |       |
|---------------------|------|-------|
| IBP                 | ° F. | 93    |
| 10%                 | ° F. | 120   |
| 30%                 | ° F. | 160   |
| 50%                 | ° F. | 202   |
| 70%                 | ° F. | 250   |
| 90%                 | ° F. | 325   |
| EP                  | ° F. | 420   |
| Reid vapor pressure |      | 11.75 |

The results of this test are as follows:

| Additive              | Concen-<br>tration,<br>percent<br>by wt. | Rating |
|-----------------------|------------------------------------------|--------|
| None                  | None                                     | 58     |
| Compound of Example 1 | 0.005                                    | 78     |
| Compound of Example 1 | 0.05                                     | 89     |

As stated heretofore, the boron compounds of this invention are stable toward hydrolysis and particularly so when dissolved in gasoline. It has been found that small amounts of these compounds may be added to gasoline as a means of improving the hydrolytic sta-

bility of other organo boron compounds which, when present in gasoline alone, have limited commercial value due to their tendency to hydrolyze in the presence of moisture. In this manner, it is possible to introduce a

desired amount of elemental boron into a gasoline by utilizing a major amount of an organo boron compound offering a high elemental boron content but otherwise undesirable due to its hydrolytic stability in conjunction with minor amounts of one or more of the boron com-

ounds of the present invention, thereby lowering the total amount of additive required in the fuel and insuring adequate hydrolytic stability. It has been found that the addition of as little as 5 to 10% of the boron additive as a compound of the class set forth hereinbefore

can significantly improve the hydrolytic stability of various organo boron compounds. This scheme of introducing adequate elemental boron to the combustion chamber to offset the adverse effects of combustion chamber deposits is particularly fortuitous since, as will be obvious from the above reported results, only very small amounts of the boron compounds of this invention are required to provide significant improvements in engine operation with respect to carburetor cleaning and carburetor anti-icing.

We claim:

1. A motor fuel for internal combustion engines consisting essentially of a leaded gasoline and from 0.0025 to 0.05% by weight of a boron compound selected from the group consisting of (1)



35 where X is selected from the group consisting of hydrogen and



and (2)



wherein  $\text{R}_x$  represents an aliphatic hydrocarbon radical containing 7 to 19 carbon atoms, where  $n$  is a small whole number from 1 to 3 and where  $\text{R}_2$  represents a radical selected from the group consisting of hydrogen and a lower alkyl radical containing 1 to 3 carbon atoms.

2. A motor fuel for internal combustion engines consisting essentially of a leaded gasoline and from 0.02 to 0.05% by weight of a compound having a formula:



65 where  $\text{R}_x$  represents an aliphatic hydrocarbon radical containing 7 to 19 carbon atoms.

3. A motor fuel for internal combustion engines consisting essentially of a leaded gasoline and from 0.02 to 0.05% by weight of a compound having a formula:



wherein  $R_x$  represents an aliphatic hydrocarbon radical containing 7 to 19 carbon atoms.

4. A motor fuel for internal combustion engines consisting essentially of a leaded gasoline and from 0.02 to 0.05% by weight of a compound having a formula: 5



10

wherein  $R_x$  represents an aliphatic hydrocarbon radical containing 7 to 19 carbon atoms.

## References Cited in the file of this patent

## UNITED STATES PATENTS

|           |                |               |
|-----------|----------------|---------------|
| 2,442,582 | Bishop         | June 1, 1948  |
| 2,450,807 | McCarthy       | Oct. 5, 1948  |
| 2,504,951 | Tryon          | Apr. 25, 1950 |
| 2,668,100 | Luvisi         | Feb. 2, 1954  |
| 2,741,548 | Darling et al. | Apr. 10, 1956 |

UNITED STATES PATENT OFFICE  
CERTIFICATION OF CORRECTION

December 20, 1960

Patent No. 2,965,459

Richard J. De Gray et al.

It is hereby certified that error appears in the above numbered patent requiring correction and that the said Letters Patent should read as corrected below.

Column 5, lines 10 to 15, the formula should appear as shown below instead of as in the patent:



Signed and sealed this 8th day of August 1961.

(SEAL)  
Attest:

ERNEST W. SWIDER  
Attesting Officer

DAVID L. LADD  
Commissioner of Patents